

# UNITED STATES PATENT OFFICE.

FRANK A. FAHRENWALD, OF CLEVELAND HEIGHTS, OHIO.

## FIREARM AND ALLOY FOR MAKING SAME.

1,346,189.

Specification of Letters Patent. Patented July 13, 1920.

No Drawing.

Application filed October 15, 1919. Serial No. 330,943.

*To all whom it may concern:*

Be it known that I, FRANK A. FAHRENWALD, a citizen of the United States, residing at Cleveland Heights, in the county of 5 Cuyahoga and State of Ohio, have invented a certain new and useful Improvement in Firearms and Alloys for Making Same, of which the following is a full, clear, and exact description.

10 This invention relates to fire arms and ordnance and has for its main objects the provision of a metallic alloy for use in the construction of the same which shall be more resistant to corrosion by the combustion products of the explosive as well as less corroded by atmospheric conditions, salt solutions, (such as sea water or perspiration) than anything now in use for the purpose; which shall compare favorably 15 with the steels at present used in respect to mechanical strength, resistance to mechanical erosion, and ease of working; which shall not be unduly high in intrinsic value; and whose coefficient of heat expanse shall be 20 very small.

It is well known that the steel ordinarily used in the manufacture of fire-arms of all calibers, such as sporting and military rifles, pistols and heavy ordnance, is easily rusted 25 by exposure to the atmosphere, is seriously corroded by ocean spray or sweaty hands, and is rapidly attacked by the combustion-products of the explosives, both solid and gaseous, especially the residues from the 30 use of smokeless powder. Firearms in which such explosives are employed must be cleaned within at least one hour after every shot in order to avoid serious pitting, which is extremely detrimental to accuracy; 35 and mere mechanical cleaning is not sufficient, but chemical means must be used to neutralize the injurious elements of the powder residue. This condition is so marked that the advertising pages of all sporting 40 and hunting periodicals of the present day are loaded with notices of cleaning compounds and solutions devised for this purpose. Furthermore, the manufacturers of gunpowders have been untiring in their 45 efforts to produce a propellant which would have no harmful after-effect on the barrel steel. I have approached this problem from a different angle, namely, that of constructing the fire-arm from a metal or alloy which 50 shall be highly resistant if not absolutely immune to these corrosive agencies. While

I have devised these alloys more particularly for the barrels, I also find them valuable in connection with the operating mechanism, particularly of automatic rifles or machine 60 guns for reasons which will hereafter appear.

As set forth in my application No. 319,822 filed August 25, 1919, the desired combination of physical and chemical properties is 65 found in alloys made by combining chromium with iron or with one or more iron-group metals, with or without other chromium-group metals. However, those alloys are more resistant chemically than is necessary for many purposes, and I have found it possible, with some saving in expense, to produce an alloy omitting chromium which will be sufficiently incorrodible for most 70 purposes and, in fact, superior in some respects. I have discovered that either pure nickel or pure cobalt is much more resistant than iron to the above-described chemical action of explosives and their residues, and that either nickel or cobalt in the forged 75 condition is of higher tensile strength and elastic limit than iron, and can be as readily machined or otherwise worked. These metals are constantly being produced in larger quantities and at lower prices, and 80 considering their higher resistance to the corroding influences met with in operation, their use at the present prices is clearly warranted in many guns. It is well known that in many sporting arms the amount of 85 metal employed is only about five pounds, and a price of from one hundred to one thousand dollars is demanded. These metals can be alloyed together in all proportions and such alloys are even superior in most 90 effects to the pure metals for use in firearms.

However, pure nickel, pure cobalt, and their alloys, possess a chemical resistivity which is needlessly high for most firearms and I have discovered that several metals 100 can be added to these with the production of alloys which still possess chemical and physical properties far superior to those of steel, and with a comparatively small intrinsic value. Thus manganese or copper or 105 both can be used up to a total of about 50% of the whole, and in combination with one or both of the metals cobalt and nickel. I find however, that iron is the most satisfactory metal with which to alloy nickel or cobalt, 110 and even when the iron is predominant, the protective effect of the other iron group

metals is still sufficiently marked to be of value in case the total proportion of iron be not greater than about 90%. When less than about 10% of nickel or cobalt (either 5 or both) is employed in conjunction with iron, it is necessary to add chromium, molybdenum, tungsten, vanadium, niobium, tantalum, titanium or zirconium in order to afford additional chemical resistance; and 10 while it is perfectly possible to do this, still the expense is considerably increased (unless by the use of some of the alloys mentioned in my former application) while such substances as titanium, zirconium, niobium 15 and tantalum have such a combined effect with carbon and silicon as to produce extreme hardness and brittleness, unless precautions are taken to restrict the carbon and silicon to extremely low limits, which is 20 itself a difficult and expensive requirement.

For certain high pressure arms, however, I find it quite advantageous to replace a part of the nickel or cobalt with substances from the titanium, vanadium, or chromium 25 groups, but keeping the iron content sufficiently high so that, with a small amount of carbon present, the alloy may be heat-treated to adjust its tensile-strength, elastic-limit, and shock-resistance.

30 As examples of alloys which I have found particularly valuable for fire-arm use I will instance the following:

- (1) Ni (and or) Co, 10%—Fe 90%.
- (2) Ni (and or) Co, 25%—Fe 75%.
- (3) Nickel 36%—Fe 64%.
- (4) Nickel (and or) Co, 50%—Fe 50%.
- (5) Nickel (and or) Co, 80%—Fe 20%.
- (6) Nickel (and or) Co, 100%.
- 40 (7) Fe—75% to 90%; Ni (or and) Co—5% to 20%; metals from the titanium or vanadium group 3% to 8%; carbon and silicon less than .5%.

45 Any of the iron group elements in the above formulæ may be replaced to a considerable extent by copper manganese, or chromium-group-metals without exceeding the limits of my invention. For example I have 50 used Monel metal with excellent results, Fe, 5; Cu, 35; Ni, 60.

55 Alloy No. 1 as above mentioned is designed more particularly for the inexpensive popular arms such as the cheaper revolvers, boy's rifles, and farmer's shot guns. For small arms the excellence of the alloys increases with increase of the nickel and cobalt content, while for heavy ordnance I esteem most highly the alloy indicated at (7). For 60 certain purposes, however, the alloy indicated at (3) above is superior to any other known composition. In the construction of double-guns (or arms with an even greater multiplicity of barrels) those barrels are 65 sometimes bored in a single block and are at

other times made separately and secured together with their bores parallel (or at a definitely predetermined angle) by brazing or soldering them rigidly together or to a common support throughout their full 70 length. It is known, in the case of double-rifles especially, that when the first barrel is fired its rise in temperature causes a sudden local thermal expansion sufficient to bend both barrels through a noticeable arc, with 75 the cooler barrel on the shorter radius, thus entirely destroying the accuracy of the arm until the temperature conditions have become equalized. A great demand exists for accurate arms of this type but the above 80 objections have hitherto prevented the demand from being supplied.

I have discovered that the very low coefficient of thermal expansion of alloys containing nickel and iron in the proportions of 85 36% to 64%, overcomes the above objection to such double-guns or plural-barreled rifles, and that by the use of this alloy it is possible not only to make a double-rifle which shall be incorrodible and untarnishable, but which 90 shall avoid the inaccuracies due to unequal expansion to which previous devices of this nature have been subject.

In automatic, self loading, or so-called "machine guns" it is also possible by the use 95 of this alloy to operate with much less clearance between moving members, and thus not only to overcome the defects known as "jamming" but also to increase greatly the accuracy of the arm. Owing to the great rise 100 in temperature of machine-guns when operated constantly over long periods, it has heretofore been necessary to make the parts very loose and with large clearances, with the result that they rattle and shake and are 105 deficient in accuracy. This nickel-iron alloy has a lower coefficient of expansion than any other known metal or alloy (excepting certain compositions of platinum and iridium 110 too expensive to be considered in this connection) and I have found that by its use, the expansion and warping of the barrel is greatly decreased and the lock and operating mechanisms will bear the same relation 115 to each other at all times, as well as being immune to corrosion by all gases, liquids, and residues met with in practice.

I have discovered that the additional of small amounts of metals from other groups than the iron group will not destroy this property, provided only that the above proportion be preserved between the nickel and the iron. Thus I may add up to, say, 10% of copper or manganese or chromium or other chromium-group metals, or up to about 125 5% of vanadium- or titanium-group metals without greatly increasing the coefficient of expansion, and with a high increase in the chemical resistivity.

These alloys may be prepared most readily 130

in small quantities by melting the pure ingredients in an electric vacuum furnace; but can also be made in large quantities without particular precautions in a furnace fired

5 with gas, fuel-oil, or coke. If the carbon and silicon be kept sufficiently low the alloys are all very ductile and may be rolled and forged at red-heat, and machined, bored, rifled, and otherwise fashioned in the same 10 manner as ordinary steel. Excess of carbon and silicon is particularly to be avoided when metals from the vanadium and titanium groups are present. Sulfur and phosphorus should be avoided in all cases.

15 All these alloys herein described and intended to be patented and secured in and by these Letters Patent are characterized by the possession of a base of iron-group metal and yet by the possession of at least about 10% 20 of some substance other than iron itself; thus securing hardness, strength, and cheapness (which the brass or bronze culverins of an earlier day did not possess), combined with incorrodibility which is lacking from 25 the steel and iron guns of the present day. These alloys are useful for and practical in all firearms from a pocket pistol to a naval gun. All the above described metals and alloys are intended to be included in the 30 claims hereto annexed nor do I restrict myself to any features or limits mentioned in these specifications except as specifically recited in the claims.

Having thus described my invention, what 35 I claim is:

1. A firearm having parts made of a metal or alloy of which at least 10% of the whole is iron-group metal and at least 10% of the whole is other than iron itself.

40 2. A firearm having parts made of a metal or alloy of which at least about 60% of the whole is iron-group metal and at least 10% of the whole is other than iron itself.

3. A firearm having parts made of a metal or alloy of which at least about 20% consists of one or more iron-group metals of 45 greater atomic weight than iron.

4. A firearm having parts made of a metal or alloy containing nickel and iron in the 50 proportion of approximately 36 parts of nickel to 64 parts of iron.

5. A firearm having parts made of a metal or alloy containing nickel and iron in the proportion of approximately 36 parts of

nickel to 64 parts of iron together with a 55 smaller proportion of a metal or metals from a group or groups other than the iron group.

6. A firearm having parts made of a metal or alloy containing at least about 10% of 60 one or more non-ferrous metals of the iron group.

7. A firearm having parts made of an alloy containing at least about 10% of one or more non-ferrous metals of the iron group 65 together with a smaller amount of one or more metals of one or more groups adjacent to the vanadium group in the periodic table.

8. A firearm having parts made of an alloy containing at least about 10% of one 70 or more non-ferrous metals of the iron group together with not more than a preponderance of one or more metals lying adjacent to the iron group in the periodic table.

9. A firearm having parts made of an al- 75loy of which at least one-fourth consists of non-ferrous metals of the iron group.

10. A firearm having parts made of an alloy containing not less than about 90% of iron-group metals of which not more than 80 about 75% of the whole is iron.

11. A multiple barreled firearm having its barrels made of an alloy containing nickel and iron in the proportion of substantially 85 36 parts of nickel to 64 parts of iron.

12. A multiple barreled firearm having its barrels made of an alloy containing between 60 and 70 parts of iron together with between 40 and 30 parts of a non-ferrous metal of the iron group. 90

13. A machine gun whose working parts are made of an alloy containing about two parts of iron to one part of a non-ferrous metal of the iron group.

14. A firearm having parts made of an 95 alloy containing a preponderance of iron group metals of which not more than about 90% of the whole is iron and which contains at least about 5% of a metal or metals from a group or groups lying between the 100 iron group and the scandium group in the periodic table, the remainder consisting of non-ferrous metals of the iron group and carbon and silicon being present to less than about 5% each. 105

In testimony whereof I hereunto affix my signature.

FRANK A. FAHRENWALD.